

Feb. 20, 1940.

T. SENDZIMIR

2,191,355

PRODUCTION OF HIGH GRADE SHEET AND STRIP  
STEEL FROM NONREFINED MOLTEN STEEL

Filed Nov. 30, 1937

2 Sheets-Sheet 1.



FIG. 1.

FIG. 2.

FIG. 3.



FIG. 4.



FIG. 5.

INVENTOR.  
TADEUSZ SENDZIMIR.

BY

Allen & Allen  
ATTORNEYS.

Feb. 20, 1940.

T. SENDZIMIR

2,191,355

PRODUCTION OF HIGH GRADE SHEET AND STRIP  
STEEL FROM NONREFINED MOLTEN STEEL

Filed Nov. 30, 1937

2 Sheets-Sheet 2



FIG. 8.



FIG. 10.

FIG. 9.



FIG. 6.



FIG. 7.

INVENTOR.

TADEUSZ SENDZIMIR.

BY

Allen & Allen

ATTORNEYS.

## UNITED STATES PATENT OFFICE

2,191,355

PRODUCTION OF HIGH GRADE SHEET AND  
STRIP STEEL FROM NONREFINED MOLTEN  
STEEL

Tadeusz Sendzimir, Paris, France

Application November 30, 1937, Serial No. 177,296  
In Germany December 3, 1936

16 Claims. (CL 29—148)

This invention relates to the production of high grade sheet and strip steel from a relatively low grade steel at a considerably reduced production cost. In conventional practice in the production of high grade sheet steel, such as automobile and deep drawing steel an especially refined material is used at the start. During the course of production further treatment is carried on in the pouring ladle and the material is subsequently carefully poured into the ingots and thereafter is hot and cold rolled to the desired finished gauge. The sheets are then annealed or normalized and subsequently pickled.

In accordance with my novel process the starting material is one of lower refining properties, in which decarbonization, deoxidation, and the removal of sulphur have not necessarily been carried as far as is usual in conventional processes. My method is based on a gradual surface refining process which is carried out during subsequent processing steps, so that the surface becomes progressively more refined, ductile and softer. Furthermore, as the strip gauge is reduced the thickness of this refined surface increases.

I prefer to pour the molten steel into rotating cylindrically shaped molds according to conventional centrifugal casting methods. The ingots thus produced are hollow and the axial length of these ingots approximates the width of the finished product. The thickness of the cylindrical wall of such an ingot may be from 20 to 100 millimeters. If proper pouring and cooling methods are used in connection with an ingot of the above mentioned thickness, segregation and liquation are substantially eliminated.

The hollow ingots after surface solidification are placed into pit furnaces of special construction where they undergo a refining process. Preferably, electric heating devices are used in order to secure a clean, dust and slag free furnace atmosphere. The proper design of the furnace and proper selection of a heat insulating material reduce the external heat requirements to a negligible value. Within this furnace a reducing and decarbonizing atmosphere is maintained. The refining process which may last several hours is predicated upon surface absorption of hydrogen and other gases which deoxidize and decarbonize the steel to a depth of several millimeters. Sulphur removal also takes place to a large degree, and it may be assumed that other reactions also take place which result in improved properties of the finished sheets. The process is gradual and is similar to the process

of carbonization by cementation. As the process continues, the refined surface skin gradually increases in thickness or in other words, the refining action penetrates more deeply into the material. For steels which need no further decarbonization the partial pressure of carbon bearing gases in the pit furnace atmosphere is increased up to the necessary balanced condition. Degassing of the ingot may be carried out by means of a partial vacuum in the pit furnace throughout the entire heat treatment or during a partial phase thereof. For this purpose there may be provided a liquid seal of molten lead at the top of the pit furnace. Thus a reduction of the surface scale and a deoxidation and decarbonization of the ingot to a depth of several millimeters may be accomplished by absorption of the gases present in the pit furnace, and thereafter by means of the above noted partial evacuation of the furnace atmosphere, a large part of the gases present in the ingot as well as newly absorbed gases may be removed.

The hollow ingots are then removed from the pit furnace in a condition in which they have been homogeneously heated to the proper rolling temperature. I have found it advantageous to select a rolling temperature which is lower than conventional rolling temperatures for the hereinafter described rolling process, thereby preventing the formation of thick or peeling scale during the short time the ingot is exposed to the atmosphere. I have found a rolling temperature from 900° C. to 1050° C. to be satisfactory. These hollow ingots may be rolled into an endless band on a special mill or they may be cut and rolled on a conventional strip mill. Preferably, the rolling processes are carried out in the absence of air or under the protection of reducing gases. The hot strips after this rolling are subsequently further refined in either coiled or flat condition. The tougher surface skin which has been provided up to this point protects the surface against possible defects during the hot rolling process, and the possibility of checking is positively prevented whereby side trimming of the strip is obviated. Furthermore, the surface of the strip is completely scale and slag free, whereby descaling processes prior and during hot rolling, as for example the squeezing of the strip or the application of high pressure water sprays, as has been found necessary in conventional methods, are thus eliminated.

In subsequent refining of a coil strip the cooling of the coil takes place in special containers which will be described hereinafter. Special pre-

caution is taken to maintain a special atmosphere in these containers. During this latter process a spontaneous annealing of the material takes place, i. e., grains which elongated during the 5 rolling processes grow and lose their directional properties. Dissolved hydrogen and other gases in the particular furnace penetrate deeper into the metal on account of the prolonged diffusion of these gases.

10 At this point in the process the thickness of the hollow ingot may be from 1.5 to 3 millimeters and above, and penetration is almost complete. If the vacuum treatment has been omitted in the pit furnace it can be added as a 15 degassing process in the strip coil annealing chamber. This latter phase of the process may also be added to produce scale free surfaces. The second vacuum treatment may be added independently of the first vacuum treatment in 20 the pit furnace. The first treatment may not produce penetration to the middle sections of the wall of the hollow ingot due to its comparative thickness at that point in the process.

An alternate process may be carried out for 25 certain grades of steel. The reducing atmosphere in the pit furnace may be provided with a carbonizing effect whereby there is produced an oxygen-free but higher carbon content surface skin.

30 The surface of the material is thoroughly decarbonized under reducing conditions in the above described cooling and annealing furnaces after the hot rolling process. At this point of the process the penetration is much deeper on 35 account of the preceding hot rolling of the strip. Decarbonization of the coiled strip during the annealing and cooling processes is considerably slower on account of impaired entrance of the gas into the strip surface. However, by virtue of the fact that rapid diffusion 40 of the carbon content in the thin and carbonized skin toward the inner part of the strip is taking place, there is produced a strip of an average carbon content which is often 45 desirable.

A further alternate process for annealing and cooling may involve the pulling of the coiled strip through a strip furnace under special atmospheres and a subsequent vacuum treatment.

50 The only difference between the second and the first process would be in the better access of the gases into the strip surfaces which would result in deeper diffusion of the gases into the metal.

55 Both processes produce a cooled strip with an absolutely clean surface whereby pickling prior to cold rolling is rendered unnecessary. Improved cold rolling is attained by the further development of the tough metal skin in

60 the annealing furnace. Checking of the strip is prevented as above pointed out, and the strip surface has far better properties than the surfaces produced by conventional methods.

The cold reduced strip is subsequently annealed or normalized. At this point of the process the invention is applied to completely deoxidize and decarbonize the strip. For this purpose strip is pulled through a furnace in which it is heated to the required annealing or 70 normalizing temperature under the influence of a suitable furnace atmosphere, and is kept at this temperature until the effect of the above described refining process has partially or completely penetrated the strip. A subsequent 75 vacuum process may be added.

The objects pointed out above and others which will be pointed out hereinafter or which will appear readily to one skilled in the art upon reading these specifications, I accomplish by that method, and by that method and apparatus of which I shall now describe certain embodiments. Reference is now made to the drawings forming a part hereof, and in which—

Figure 1 shows central vertical cross section of a pit furnace for processing the hollow ingots 10 prior to hot rolling.

Fig. 2 is a view similar to Fig. 1 showing the manner in which the ingots may be charged into and removed from the furnace.

Fig. 3 is a diagrammatic plan view showing a 15 desirable arrangement of pit furnaces.

Fig. 4 is a cross sectional view of a furnace used in connection with the hot rolling of the ingot taken on the line 4—4 of Fig. 5.

Fig. 5 is a longitudinal cross sectional view taken on the line 5—5 of Fig. 4 and showing a 20 two high hot mill in connection with the furnace.

Fig. 6 is a central vertical cross section showing another arrangement of a furnace and mill 25 in which the ingot is shown in an early phase of the rolling process.

Fig. 7 is a view similar to Fig. 6 showing the 30 rolling during a later phase of the process.

Fig. 8 is a vertical longitudinal section of a 35 cooling chamber for the hot rolled and coiled strip.

Fig. 9 is a detailed cross sectional view similar to Fig. 8 showing the sealing arrangement for 35 the chamber bell.

Fig. 10 is a view similar to Fig. 8 of a modification of the cooling chamber.

The pit furnace shown in Figs. 1, 2 and 3 comprises an insulating base 9, a base plate 8 and walls 21. A desirable honeycomb arrangement of the individual pits is shown in Fig. 3. The hollow ingot 1 rests on a member 2, which may be a ring or a number of blocks annularly disposed. A cylinder 3 is located internally of the ingot to provide support for the lid 17 and 45 the heating elements 4. A cylindrical shell 15 provides additional support for the furnace walls 21 and also serves in connection with a liquid seal indicated generally at 13. The lid 17 is provided with an outer cover or bell 14 which 50 dips into the liquid seal. The atmospheric pressure within the furnace chamber may be lowered by the selection of a relatively high outer bell member 14 whereby a higher sealing liquid level may be obtained on the inner side of the member 14, as indicated at 16. Where it is not necessary to maintain a pressure difference within the furnace other types of seals such as dust seals 55 may be used.

The wires 6 provide leads for the heating elements 4. Leads 6 make contact with current connectors which may advantageously be arranged in a trench 7. The pipes 5 and 11 are inlet and outlet connections respectively for the 60 processing gases, and the pipe 10 is provided for removal of gas to permit a reduction of the gas pressure within the furnace.

In accordance with my process, when that phase thereof which is conducted in the pit furnace is completed, the pressure within the furnace is brought to atmospheric pressure and the lid 17 is removed by a crane. The lifter 20 is then lowered into the pit and the hooks 19 thereof are turned and engaged under the ingot which is then removed from the furnace and quickly 75

fed into the hot mill. The use of the member 20 will be clear from a consideration of Fig. 2. Since the hooks 19 fill most of the available space between the cylindrical shell 15 and the ingot 1, a proper balancing of the ingot during charging and removal thereof into and from the furnace is insured.

In Figs. 4 and 5, I have shown an element for hot rolling the pre-processed hollow ingot. A mill 30 is provided with working rolls 31, 32, and a drive which is not shown inasmuch as it forms no part of my invention. Mechanism is also provided (not shown) for feeding the hollow ingot into the mill. This may be accomplished by removing one of the working rolls or a roll bearing. The looping roll 34 may be removed by an axial motion. Directly beneath the working rolls I have provided a roller table 35, so that as the cylindrical ingot is reduced, it will gradually touch the roller table 35. If the loop being rolled is touching the roller table 35, it will be clear that if the rotation of the mill rolls is as shown in Fig. 5, an increase in the speed of the roller table 35 will cause a loop to form toward the left side of the mill, so that when the loop has grown sufficiently the roller 34 may be inserted into the loop. Thereupon the speed of the roller table is reduced below the peripheral speed of the working rolls, whereby the loop in its further growth will form toward the right hand side of the mill, whereby the roller 41 may ultimately be introduced into the loop.

I have indicated generally at 36 a furnace for holding the heat of the strip during the rolling process. This furnace may be provided with a reducing atmosphere so that a reducing process may take place at the same time as the rolling process, and by means of a lowered furnace temperature, surface oxidation of the strip is prevented. Insulating walls are shown at 44 and 45, and the furnace is provided with rails 43 for the carriages 42 upon which is mounted a freely turning roller 41. A mechanism for moving the carriages 42 in the furnace is provided by means of the chain 40 and the sprockets 39 and 48 driven by the motor 49.

For heating the furnace I prefer to provide sectional heating elements 46. Suitable gas is fed into the furnace through the pipe 47. The front wall 50 of the furnace is made quickly removable for the purpose of introducing the strip into the furnace. In charging the furnace when the loop of the strip has grown to a sufficient size, the front wall 15 is removed and the roller 41 is run out of the furnace by means of its carriages 42. The roller 41 is then removed from the carriages 42, inserted into the rapidly forming loop in the endless strip and replaced on the carriages. The assembly is then pulled back into the furnace by means of the chains 40. The roller 41 is pulled back into the furnace until the strip loop is raised from the roller table 35. The front wall 50 is then replaced. It will be noted that this front wall is provided with seals 37 and 38 for the upper and lower flight of the strip. It will, of course, be understood that if necessary or desirable, the strip may be put under tension. The operations outlined immediately above must be done very rapidly in order to eliminate gas loss and interruption of the rolling process. When the rolling process is complete, the strip 33 is cut and subsequently coiled.

In Figs. 6 and 7 I have shown an alternate arrangement in a rolling mill and furnace for rolling hollow ingots. In these figures I have shown

a three high mill 60 in which the rolling pass is between the middle roll 62 and the bottom roll 63. Directly under the mill I provide a roller table 73 with an adjustable speed drive. This table comprises a stationary section 64 and a movable section 65. Immediately below this table I provide a pit furnace indicated generally at 68, and provide it with suitable heating elements 67. Although the furnace may be heated by glow pipes or open flame, I prefer to provide electric heating elements because a reducing atmosphere free from ashes, slag and other deleterious constituents is desired, so that the surface properties of the strip will not be impaired. A suitable atmosphere may be provided within the furnace by leading into it an appropriate gas by means of the pipe 70. It may be satisfactory to use internal combustion motors such as Diesel motors for the mill drives, and in such cases the exhaust gases of these motors may be fed directly through the pipe 70 alone or mixed with other gases. Such mill drives can produce sufficient amounts of exhaust gas for this process, not only for the furnace requirements during hot rolling, but for furnaces utilized in the later processing of the strip.

When the strip 66 has reached a sufficient length, the removable section 65 of the roller table is moved so as to permit the strip to hang freely within the furnace, as shown in Fig. 7. It will be noted that the only portion of the furnace which is open to the atmosphere is the relatively narrow opening at the top, and this passage is sealed from the atmosphere by means of flame sheets 74 provided by the burners 73, whereby the entire process is carried out under the effect of a protecting gas.

I have provided mechanically driven rollers 75, whereby upon completion of the rolling process, the strip 66 may be lifted out of the pit furnace 40 so that it may be cut by means of the shears 72 and coiled upon the coiler 71 located conveniently adjacent the mill 60. After coiling, the strip which is at a relatively high temperature of approximately 700 to 800° C. is fed into a cooling apparatus.

Referring now to Figs. 8, 9, and 10 which show two modifications of a cooling apparatus in which the strip is cooled in a special atmosphere and if desired under partial vacuum prior to a subsequent cold rolling operation. In Fig. 8 a base 91 is provided with grooves for providing a liquid seal. The coils 81 are set onto pads 82 and covered with lids 80. These lids are preferably provided with an insulating lining 86 in order to prolong the cooling process. The ring 87 supports the lining 86 and the flexible angle 89 provides in conjunction with the liquid 90 the necessary seal during the removal of the gas from the lid 80 through the pipe 85. Gas inlet and outlet pipes are shown respectively at 83 and 84, and these may also be used to flush the chamber with a suitable gas. In Fig. 10 I have shown an alternate arrangement in which a fluid seal is provided which will permit of partial evacuation of the annealing chamber. For this purpose, of course, the sealing liquid must extend considerably higher than in the other case. But generally speaking, the principles of the devices of Figs. 8 and 10 are the same.

Other arrangements may also be used for cooling the strips. In some instances, particularly in cases where the finished temperature of the rolling process is too low, it is advantageous to conduct the strip directly through a heating

furnace with a corresponding cooling chamber, so that the strip is re-heated and then cooled. With this latter arrangement a better access of the special atmosphere into the strip surface is accomplished.

The hereinabove described refining process and modification of the contents of various constituents, as for example, carbon, sulphur gases, etc., with the diffusion method may be advantageous-

10 ly applied to other processing methods. For example, a bi-metallic ingot can be produced by pouring small amounts of dissimilar metal into the r tating mold. Alternatively the inner surface of the mold may be covered with the dis-

15 similar metal, such as chromium, copper, nickel, aluminum and other metals, either individually or in alloyed form. Or the inner surface of such mold may be lined with a paste containing such metal or metals either free or chemically bound.

20 It may also be heat-insulated, to make the adsorption of such alloy metals more complete. These metals fully dissolved by the liquid parent metal or partially dissolved by the solidified parent metal, will form an alloy skin on the surface

25 of the hollow ingot. The above described further processing in the pit furnace produces a further advantageous diffusion under reducing conditions, as well as the addition of gases which advantageously effect the quality and properties of

30 the skin, with respect to, for example, corrosion resistance. Subsequent processing of the coils in the annealing and cooling furnaces leads to a partial absorption of the alloy metal on the other side of the strip, whereby an alloy skin is provided on both sides thereof.

Modifications may be made in my invention without departing from the spirit thereof, and I do not intend to limit myself otherwise than as pointed out in the claims which follow.

40 Having thus described my invention, what I claim as new and desire to secure by Letters Patent is:

1. A process for the production of refined steel strip of fine gauges from a less refined molten metal, which includes the steps of producing an ingot of relatively thin section and preferably hollow shaped, and subjecting said ingot to an initial heat treating operation under the influence of a reducing atmosphere in a furnace, then to a 45 rolling operation in a mill, and thereafter alternating heat treating operations with rolling operations to obtain a further refinement of the metal by a combined atmosphere and temperature action upon the said metal, improving chiefly the condition of the surface layer of metal 50 while on account of said rolling operations, said surface layer increases in relation to the weight.

2. A process of producing refined steel stock of fine gauges in accordance with claim 1, which includes the step of reducing the stock in the form 60 of an endless belt and passing said belt through a chamber containing reducing gases.

3. A process for producing rolled metal stock which comprises centrifugally casting molten 65 metal to form a hollow ingot, heat treating said hollow ingot, inserting said ingot over a roll of a rolling mill, rolling said ingot in said mill, and during said rolling causing the metal being rolled to pass over an additional stationary roll and an 70 additional movable roll, and applying force to said movable roll to exert a tension on said metal while being rolled.

4. A process for producing rolled metal stock which comprises centrifugally casting molten metal to form a hollow ingot, heat treating said

hollow ingot, inserting said ingot over a roll of a rolling mill, rolling said ingot in said mill, and during said rolling causing the metal being rolled to pass over an additional stationary roll and an additional movable roll, and applying force to said movable roll to exert a tension on said metal while being rolled, cutting and coiling the metal after rolling, and further refining said metal by heat treating it in the presence of a reducing gas.

5. A process for producing rolled metal stock 10 which comprises centrifugally casting molten metal to form a hollow ingot, heat treating said hollow ingot, inserting said ingot over a roll of a rolling mill, rolling said ingot in said mill, and during said rolling causing the metal being rolled 15 to pass over an additional stationary roll and an additional movable roll, and applying force to said movable roll to exert a tension on said metal while being rolled, maintaining a portion 20 of the metal during rolling under heat in a reducing atmosphere, and finally cutting and coiling the metal after rolling, and further refining said metal by heat treating it in the presence of a reducing gas.

6. A process for the production of refined steel strip of fine gauges from less refined metal which includes the steps of producing an ingot of a relatively thin section and rolling it in successive steps to the desired gauge, forming at least before the first rolling step a refined surface layer 30 on the processed stock by heating it in the presence of a reducing gas for sufficient length to form a layer which completely encloses said stock, and through its improved rolling qualities 35 protects the cohesion of the less refined metal during said rolling operations.

7. A process of producing strip by rolling from cast metal relatively high in impurities and normally unsuitable for rolling, which comprises casting a thin-walled ingot from said metal, then heat-treating said ingot under a reducing atmosphere for a sufficient length of time and at a sufficient temperature to refine a surface layer of said metal ingot, then transferring said ingot to a mill and hot rolling it.

8. A process of producing strip by rolling from cast metal relatively high in impurities and normally unsuitable for rolling, which comprises casting a thin-walled ingot from said metal, then heat-treating said ingot under a reducing atmosphere for a sufficient length of time and at a sufficient temperature to refine a surface layer of said metal ingot, then transferring said ingot to a mill and hot rolling it in a plurality of passes, and intermediate said passes protecting surface layers of said metal by heat treating it in a reducing atmosphere.

9. A process of producing strip by rolling from cast metal relatively high in impurities and normally unsuitable for rolling, which comprises casting a thin-walled ingot from said metal, then heat-treating said ingot under a reducing atmosphere for a sufficient length of time and at a sufficient temperature to refine a surface of said metal ingot, then transferring said ingot to a mill and hot rolling it, said heat treatment being concluded with a treatment under a reduced pressure whereby to remove from said surface layer of the metal absorbed gases.

10. A process of producing strip by rolling from cast metal relatively high in impurities and normally unsuitable for rolling, which comprises casting a thin-walled ingot from said metal, then heat-treating said ingot under a reducing atmosphere for a sufficient length of time and at a

- sufficient temperature to refine a surface layer of said metal ingot, then transferring said ingot to a mill and hot rolling it in a plurality of passes, and intermediate said passes protecting surface 5 layers of said metal by heat treating it in a reducing atmosphere, finally heat treating the hot-reduced strip in a reducing atmosphere to further refine it, and further reducing the strip by cold rolling.
- 10 11. A process of producing strip metal from a metal normally unsuitable for rolling and relatively high in impurities, which comprises casting said metal to form a hollow ingot, then heat treating said ingot in a furnace under a reducing atmosphere at sufficient temperature and for a sufficient length of time to refine a surface layer of said metal so that the ingot may be hot rolled, then transferring said ingot to a mill, placing it over a roll thereof, and hot rolling 15 said ingot to strip form.
12. A process of producing strip metal from a metal normally unsuitable for rolling and relatively high in impurities, which comprises casting said metal to form a hollow ingot, then heat 20 treating said ingot in a furnace under a reducing atmosphere at sufficient temperature and for a sufficient length of time to refine a surface layer of said metal so that the ingot may be hot rolled, then transferring said ingot to a mill, placing it over a roll thereof, and hot rolling 25 said ingot to strip form and while so hot rolling said ingot causing a portion thereof to lie within a heated furnace having a reducing atmosphere.
13. A process of producing strip metal from a metal normally unsuitable for rolling and relatively high in impurities, which comprises casting said metal to form a hollow ingot, then heat 30 treating said ingot in a furnace under a reducing atmosphere at sufficient temperature and for a sufficient length of time to refine a surface layer of said metal so that the ingot may be hot rolled, then transferring said ingot to a mill, placing it over a roll thereof, and hot rolling 35 said ingot to strip form and while so hot rolling said ingot
- causing a portion thereof to lie within a heated furnace having a reducing atmosphere, finally shearing and coiling the strip material so formed, heat treating it in a reducing atmosphere so as to increase the ratio of the thickness of the refined skin to the total thickness, and cold rolling the thus treated strip, then again annealing it in a reducing atmosphere to further increase the said ratio.
14. Process for refining steel according to claim 10 1 including a heat treatment of the steel ingot in a heat treating chamber adapted to withstand high temperatures and with a gas-tight seal and connections for the supply and evacuation of gases and consisting in bringing it in contact for a while with suitable gases preferably circulating while at an elevated temperature and immediately afterwards evacuating the greatest portion of said gases thereby creating a partial vacuum in said heat treating chamber and so causing most of the gases used for the treatment and which became absorbed in said steel ingot, to escape.
15. Process for refining steel according to claim 15 20 including the step of hot-reducing the steel ingot in the form of an endless belt and passing said belt through a chamber containing non-oxidizing gases, which step consists of supplying said object to the mill from a chamber filled with non-oxidizing gases and withdrawing it from said mill into a similar chamber while protecting it from oxidation on its way to and from the mill and while in said mill by flame walls.
16. Process for refining steel according to claim 25 30 1 including the step of rolling the ingot in the form of an endless belt and passing said belt through a chamber containing non-oxidizing gases, in which process the step of hot rolling is first carried out without protective atmosphere as long as the steel object is relatively thick and stiff, and afterward a part of the metal is allowed to run through said chamber having a non-oxidizing atmosphere.

TADEUSZ SENDZIMIR.